

March 6, 1962

G. S. FOERSTER

3,024,108

MAGNESIUM-BASE ALLOY

Filed Feb. 19, 1960



INVENTOR.

George S. Foerster

BY

Edward E. Schelling

AGENT

1

3,024,108

## MAGNESIUM-BASE ALLOY

George S. Foerster, Midland, Mich., assignor to The Dow Chemical Company, Midland, Mich., a corporation of Delaware

Filed Feb. 19, 1960, Ser. No. 9,936

8 Claims. (Cl. 75—168)

This invention relates to magnesium-base alloys. It more particularly concerns an improved magnesium-base alloy containing zinc and manganese.

The beneficial effects obtained upon alloying zinc with magnesium are well known. However, attempts to develop a magnesium-base alloy containing zinc and manganese which possesses, in rolled form, good longitudinal and transverse properties in both directions of rolling have heretofore been unsuccessful. Magnesium-zinc-manganese alloys have shown poor rollability when the zinc content exceeds about 3 percent. Magnesium-base magnesium-zinc-manganese alloys containing less than about 3 percent of zinc have been satisfactorily hot rolled but at the same time have exhibited poor cold workability, and as the zinc content is decreased, the alloys in rolled form possess increasingly poorer mechanical properties. The poor properties of conventional magnesium-base magnesium-zinc alloys are believed due to heterogenous deformation which occurs when the alloy is strain hardened as by cold rolling.

It is the principal object of the invention to provide an improved magnesium-base alloy containing both zinc and manganese which is readily rollable and which in rolled form exhibits desirably high tensile and compressive properties in both the longitudinal and transverse directions of rolling.

Other objects and advantages of the invention will become apparent as the description of the invention proceeds.

The invention is based on the discovery that in certain limited ranges of proportions of zinc and manganese, herein shown, the addition of rare earth metal to the magnesium-base alloys containing these metals greatly improves their properties. In particular it has been found that in magnesium-base alloys containing from 1.25 to 3 percent of zinc (preferably 1.75 to 2.5 percent), and from 0.1 to 2 percent of manganese (preferably 1 to 2 percent), the addition of a critical amount of rare earth metal, the amount by weight being from 0.04 to 0.2 as much rare earth metal as zinc, the balance being magnesium, a magnesium-base alloy is obtained which in rolled form exhibits good ductility, toughness, formability, resistance to corrosion, and satisfactory weldability without stress relief and the rolled products have substantially the same high tensile and compressive strengths in both the longitudinal and transverse directions of rolling. The invention then consists of the improved magnesium-base alloy herein described and particularly pointed out in the claims.

The addition of rare earth metals, which ordinarily adversely affect extrudability and room temperature mechanical properties of magnesium-zinc alloys in cast form, is decidedly beneficial to the magnesium-zinc alloys in rolled form. Rare earth metal additions improve hot rollability of the high zinc alloys, apparently by decreasing the concentration of the low-melting magnesium-zinc phase(s) and markedly improve cold workability and resultant properties, apparently through promotion of more homogeneous deformation. However, the proportion of rare earth metal added is critical and the addition of too much rare earth metal adversely effects transverse strength, formability, and mechanical properties generally.

A notable feature of the addition of rare earth metal in the critical concentration range herein disclosed is the effect on the longitudinal and transverse properties of the

2

alloy in rolled form. The transverse properties of the said magnesium-zinc-manganese alloys are quite generally higher than the longitudinal properties. Yet upon making small, but increasingly larger additions, to a typical example of the said Mg-Zn-Mn alloy, of rare earth metal covering the said critical concentration range, the longitudinal properties of the resulting compositions in rolled form are found respectively to be successively larger while at the same time the transverse properties respectively are found successively to approach a maximum value and then to decrease to values smaller than that of the longitudinal properties. The compositions in the range in which the values of the longitudinal and transverse properties of the alloy approach, become equal, and diverge slightly are those herein disclosed and claimed.

It has not been previously shown that upon varying the proportions of a minor component of an alloy the relative magnitudes of the transverse and longitudinal properties are reversed. Nor is it expected in the art that such a change is produced by such small changes in the proportions of a minor component.

As the zinc content of the alloy is increased, the amount of rare earth metal needed to bring about the transposition of the magnitudes of transverse and longitudinal properties of the alloy is proportionately increased. To produce an alloy having the desired combination of properties, it is therefore necessary to add an amount of rare earth metal proportionate to the zinc content. Suitable rare earth metal to zinc ratios for the present alloy are those from 0.04 to 0.2 and preferably from 0.06 to 0.12. These ratios are illustrated graphically in the appended drawing.

In the drawing the single figure shows a rectangular coordinate graph in which percent zinc is plotted along the ordinate scale and percent rare earth metal is plotted along the abscissa. The range of proportions of rare earth metal and zinc in the alloy herein disclosed and claimed is graphically represented by the closed area bounded by the lines connecting points A, B, C and D, said alloy including from 0.1 to 2 percent of manganese and the balance magnesium. The preferred range of proportions of rare earth metal and zinc is graphically represented in the same drawing as the closed area bounded by the lines connecting points E, F, G and H.

Again referring to the drawing, magnesium-zinc-manganese-rare earth metal alloys in rolled form and (1) having rare earth metal-zinc ratios corresponding to the region generally below the line AD exhibit low mechanical properties (2) having ratios corresponding to the region to the right of the line CD generally exhibit low transverse properties, (3) having ratios corresponding to the region above the line BC exhibit poor rollability and weldability, and (4) having ratios corresponding to the region to the left of the line AB exhibit low longitudinal properties and poor rollability.

The rare earth metals suitable for use in preparing the present alloy are: cerium, lanthanum, praseodymium, neodymium or misch metal. Misch metal with from 35 to 80 percent of cerium, the balance being rare earth metal and up to 5 percent of non-rare earth metal, is the preferred rare earth metal ingredient of the alloy. Any of the foregoing rare earth metals may be used alone or in any combination in compounding the alloy.

If desired, thorium may be substituted for all or a portion of the rare earth metal content of the alloy with no loss in properties. Substitution by thorium, however, is on the basis of an equal atomic percent which corresponds on a weight basis to the use of an amount of thorium equal to about 1.6 times the weight of the rare earth metal replaced.

The alloy may be made in the desired proportions according to the invention by melting together the alloying

ingredients in proper proportions or by using hardeners of magnesium alloys containing the alloy constituents. Protection from oxidation during alloying is effected by the use of a magnesium chloride-free saline flux as in conventional alloying. The molten alloy may be flux refined by stirring the alloy with additional flux. The so-refined alloy is allowed to settle and then is separated from the flux as by decanting into a suitable casting mold, e.g., a slab mold for rolling stock.

Zirconium, in the form of a magnesium-zirconium hardener, or master alloy, may be advantageously added

5 These rolling slabs were scalped to about  $1\frac{1}{8}$  inches thickness, heated to about  $800^{\circ}$  to  $850^{\circ}$  F. and cross-rolled to a thickness of about 1 inch, then turned 90 degrees and rolled to about  $\frac{1}{8}$  inch thickness, and annealed for one hour at  $700^{\circ}$  F. The annealed strips were then cold rolled in multiple passes at 1 to 2 percent per pass to a thickness of about 0.1 inch, then annealed for one hour at  $700^{\circ}$  F. and cold rolled an additional 40 percent. The rolled strip was finally heat treated for one hour at  $275^{\circ}$  F. The properties set forth in Table 1 were determined on the so-prepared rolled strip.

Table 1

| Alloy No. | Percent composition, bal. Mg |       |       |     | Properties of the alloy in rolled form |     |     |    |            |     |     |    |
|-----------|------------------------------|-------|-------|-----|----------------------------------------|-----|-----|----|------------|-----|-----|----|
|           |                              |       |       |     | Longitudinal                           |     |     |    | Transverse |     |     |    |
|           | Zn                           | MM    | Th    | Mn  | Percent E                              | TYS | CYS | TS | Percent E  | TYS | CYS | TS |
| 1         | 1.4                          | .12   | ----- | .95 | 6                                      | 34  | 33  | 43 | 16         | 31  | 32  | 44 |
| 2         | 1.4                          | .12   | ----- | 1.9 | 6                                      | 35  | 34  | 45 | 14         | 32  | 33  | 45 |
| 3         | 1.5                          | .10   | ----- | 1.5 | 7                                      | 36  | 35  | 46 | 18         | 33  | 33  | 46 |
| 4         | 2.0                          | .12   | ----- | 1.6 | 7                                      | 37  | 37  | 46 | 13         | 36  | 38  | 48 |
| 5         | 2.5                          | .25   | ----- | 1.5 | 7                                      | 37  | 37  | 46 | 13         | 36  | 38  | 48 |
| 6         | 2.2                          | .11   | .15   | 1.5 | 6                                      | 40  | 36  | 49 | 16         | 35  | 37  | 49 |
| 7         | 2.2                          | ----- | .26   | 1.5 | 5                                      | 35  | 30  | 43 | 12         | 40  | 39  | 50 |

Percent E = percent elongation.

TYS = tensile yield strength, at 0.2 percent deviation from the modulus line.

CYS = compressive yield strength, at 0.2 percent deviation from the modulus line.

TS = ultimate tensile strength.

All strengths listed in thousands of p.s.i.

MM = misch metal used consisted of 48% Ce, 18% Nd, 5.5% Pr, and 28.5% La which included minor amounts

of other rare earth metals.

to the melt, prior to the settling stage, to improve the malleability of the alloy in rolling slab form. An amount of zirconium by weight from 0.001 to 0.05 percent of the weight of the alloy is effective. Larger amounts of zirconium are to be avoided as likely to cause precipitation of part of the desired manganese content of the alloy.

In rolling the cast metal, it is desirable first to scalp the cast metal so as to present a smooth clean surface to the rolls of the rolling mill. The clean rolling stock is heated to a suitable rolling temperature, e.g., about  $800^{\circ}$  to  $850^{\circ}$  F. The heated metal is then reduced in thickness by passes between the rolls of the mill, the rolling being stopped 50 to 100 Fahrenheit degrees short of the temperature at which cracking would result if the rolling were continued without reheating the metal. The temperature to which the metal may decline as it is being rolled before cracking occurs is readily determined by trial and varies with the proportions of the alloying ingredients. In general in hot rolling, the metal should be reheated when its temperature declines to about  $600^{\circ}$  or  $650^{\circ}$  F., if rolling is to be continued without cracking. Reductions in thickness of the cast metal of 20 to 30 percent may be made per pass while the metal is at a suitable rolling temperature.

By annealing the hot rolled cast metal, as for example, by heating for one hour at  $700^{\circ}$  F., the hot rolled metal may be cold rolled (warm rolls, e.g.,  $180^{\circ}$  F.) as much as 40 to 50 percent by making thickness reductions of 1 to 2 percent per pass. Before proceeding with the final 40 to 50 percent cold reduction by rolling, it is generally desirable to use a preliminary total cold roll of about 15 percent, obtained in multiple passes, followed by annealing at about  $700^{\circ}$  F. for one hour to improve the subsequent cold rollability and mechanical properties.

Examples of the alloy according to the invention were cast in rolling slabs 2 inches by 4 inches by 8 inches.

45 Compositions of the alloy containing about 2 percent or more of zinc are desirably worked, as by extruding, before forming into rolled products. Extrudes, of these compositions, in the form of slabs make desirable rolling stock and permit making rolled products by either hot or cold rolling. For example, for making rolled products, ingot of the alloy is heated to and extruded at about  $600^{\circ}$  and  $800^{\circ}$  F. depending upon the amount of reduction to be made. That is, for high reductions the higher temperatures of the range are used; small reductions may 50 be made at the lower temperatures of the range. Prior to rolling, the extrude (slab) is heated to between about  $800^{\circ}$  and  $850^{\circ}$  F. for example. The heated extrude is rolled in a number of passes without reheating until the metal requires reheating to avoid cold cracking. On annealing the hot rolled product so obtained, for one hour at about  $700^{\circ}$  F., for example, it may be cold rolled (warm rolls  $180^{\circ}$  F.) as much as 45 to 50 percent thinner. The data in Table 2 set forth specific examples of the alloy and their properties in the form of pre-extruded 55 rolled strip.

60 In making this rolled strip, four ingots, each of a different alloy, were cast into three inch diameter billets. These were machined to a diameter of  $2\frac{15}{16}$  inches, heated to  $750^{\circ}$  F., then extruded at  $700^{\circ}$  F. into strip  $\frac{3}{8}$  inch by 2 inches for rolling stock. The extruded strip was heated to  $800^{\circ}$  F., cross-rolled in several passes to a thickness of  $\frac{3}{16}$  inch, turned and rolled parallel to the direction of extrusion to a thickness of about 0.1 inch, reheated, and rerolled at  $850^{\circ}$  F. in one pass to a thickness of  $\frac{1}{16}$  inch. The rolled strip was annealed for one hour at  $700^{\circ}$  F. The annealed strip so obtained was cold rolled about 1 to 2 percent thinner per pass, the total cold reduction being about 40 percent. The cold rolled strip was heat treated one hour at  $275^{\circ}$  F., then the properties set forth 65 in Table 2 were determined.

Table 2

| Alloy No. | Percent composition,<br>balance Mg |      |     | Properties of pre-extruded rolled alloy |     |     |    |            |     |     |    |
|-----------|------------------------------------|------|-----|-----------------------------------------|-----|-----|----|------------|-----|-----|----|
|           |                                    |      |     | Longitudinal                            |     |     |    | Transverse |     |     |    |
|           | Zn                                 | MM   | Mn  | Percent E                               | TYs | CYS | TS | Percent E  | TYs | CYS | TS |
| 8-----    | 2.3                                | 0.2  | 1.6 | 6                                       | 36  | 37  | 46 | 13         | 34  | 37  | 48 |
| 9-----    | 2.5                                | 0.1  | 1.5 | 5                                       | 36  | 36  | 46 | 14         | 36  | 38  | 49 |
| 10-----   | 3.0                                | 0.15 | 1.5 | 6                                       | 35  | 34  | 45 | 12         | 35  | 36  | 48 |
| 11-----   | 3.0                                | 0.45 | 1.5 | 8                                       | 35  | 36  | 45 | 14         | 33  | 34  | 47 |

Percent E = percent elongation.

TYs = tensile yield strength, at 0.2 percent deviation from the modulus line.

CYS = compressive yield strength, at 0.2 percent deviation from the modulus line.

TS = tensile strength.

All strengths listed in thousands of p.s.i.

MM = misch metal used consisted of 48% Ce, 18% Nd, 5.5% Pr, and 28.5% La which included minor amounts of other rare earth metals.

Among the advantages of the invention are that an alloy is provided having the light weight characteristic of magnesium and possessing formability, corrosion resistance and good weldability.

This is a continuation-in-part of my copending application Serial No. 746,411, filed July 3, 1958, now abandoned.

I claim:

1. A magnesium-base alloy consisting of from 1.25 to 3 percent of zinc, from 0.1 to 2 percent of manganese, and rare earth metal in an amount in percent by weight which is from 0.04 to 0.2 of the zinc percentage, the balance of the alloy being magnesium.

2. The alloy as in claim 1 in which the rare earth metal is misch metal.

3. The alloy as in claim 1 in which up to 100 percent of the rare earth metal content is replaced by thorium, the amount of thorium by weight being about 1.6 times the weight of rare earth metal replaced.

4. A magnesium-base alloy consisting of from 1.25 to 3 percent of zinc, from 1 to 2 percent of manganese, and rare earth metal in an amount in percent by weight which is from 0.04 to 0.2 of the zinc percentage, the balance of the alloy being magnesium.

5. A magnesium-base alloy consisting of 1.75 to 2.5 percent of zinc, from 1 to 2 percent of manganese, and rare earth metal in an amount in percent by weight which is from 0.04 to 0.2 of the zinc percentage, the balance of the alloy being magnesium.

6. A magnesium-base alloy consisting of 1.75 to 2.5 percent of zinc, from 1 to 2 percent of manganese, and rare earth metal in an amount in percent by weight which is from 0.06 to 0.12 of the zinc percentage, the balance of the alloy being magnesium.

7. The alloy as in claim 6 in which up to 100 percent of the rare earth metal content is replaced by thorium, the amount of thorium by weight being about 1.6 times the weight of rare earth metal replaced.

8. A magnesium-base alloy containing about 2 percent of zinc, 0.15 percent of misch metal, and about 1.5 percent of manganese, the balance being magnesium.

## References Cited in the file of this patent

## UNITED STATES PATENTS

- 2,788,272 Whitehead et al. \_\_\_\_\_ Apr. 9, 1957  
 2,829,973 Jessup et al. \_\_\_\_\_ Apr. 8, 1958